

F. CUTTER.

PROCESS OF MAKING INGOTS.

APPLICATION FILED APR. 23, 1908.

899,827.

Patented Sept. 29, 1908.



FIG. 1.



FIG. 2.



FIG. 3.



FIG. 4.

WITNESSES.

C. T. Hannigan.  
Joseph E. Burns.

INVENTOR

Frank Cutter  
By Horatio E. Bellows  
Attorney.

# UNITED STATES PATENT OFFICE.

FRANK CUTTER, OF PROVIDENCE, RHODE ISLAND.

## PROCESS OF MAKING INGOTS.

No. 899,827.

Specification of Letters Patent. Patented Sept. 29, 1908.

Application filed April 23, 1908. Serial No. 428,765.

To all whom it may concern:

Be it known that I, FRANK CUTTER, a citizen of the United States, residing at Providence, in the county of Providence and State 5 of Rhode Island, have invented certain new and useful Improvements in Processes of Making Ingots, of which the following is a specification.

My invention relates to compound ingots adapted to be reduced into seamless plated wire for jewelers' use. The usual method of constructing these ingots has been to insert a base metal core into a precious metal tube, interpose solder of some form between 10 the contacting surfaces and subject to heat to fuse the intermediate solder sheet. Another method proposed is to "sweat" the core and shell together. That is, rely upon the fusion of the constituent parts of the core 15 and shell to unite the same. None of these enumerated processes have been satisfactory, since they all involve a micrometric fitting of the core and shell prior to the uniting step, which involves great time and expert 20 skill to perform, but the ingot and resulting wire was ruined by "blisters." These blisters always result above an area where air occurs between the core and shell, by reason 25 of the uneven flow of solder, or imperfect 30 grinding of contacting faces, or the contact of an operative's finger with the surface of the core or shell before assembling. It has been difficult to so measure and construct the precious metal shell as to be assured that the 35 thickness of its wall will be uniform throughout its area.

To the end essentially of overcoming the above enumerated disadvantages, and of securing a perfect and uniform product, and at 40 a minimum of expense and labor, my improved process consists in the steps herein-after set forth and claimed.

In the drawings which form a part of this specification, Figure 1 is a perspective view 45 of a base metal core or rod before electro-deposition. Fig. 2, a similar view of the same after the coating or deposit of precious metal thereto, Fig. 3, a like view of the completed ingot, and Fig. 4, a like view of a hollow core.

Like reference characters indicate like parts throughout the views.

In the drawings, A represents a rod or core 50 of base metal or composition, upon which I deposit by the common method of electro-

plating a coat, layer, skin, or film, B, of precious metal, such as gold or silver. After the electroplating step it will be found that the film, B, is more or less granular in character, soft, and not sufficiently adhesive to 60 the rod, A, for the purposes of seamless wire. The rod with its surrounding skin is next treated by impact, or in other words, it is subjected to beating, pressure, or hammering, which is uniform in force over the whole area 65 of the rod. By this means, the granular character of the deposit, B, is changed, the film is hardened, its surface is smoothed, and a perfect adherence of the skin to the rod, B, secured. A successful method of performing 70 this step is by forcing or precipitating shot or other metal objects against the skin, either by gravity or machinery. When shot are employed, I prefer to place the coated rod in an ordinary rattling barrel or drum containing shot, and rotate the drum; by which means the desired ends are attained. A more polished surface is secured by mixing with the shot a liquid soap. If a thin plating 75 of metal is all that is desired, the ingot is now 80 complete and ready for reduction to seamless wire by any of the usual methods for that purpose. If a heavier plate is demanded, the above described plating and beating steps 85

In constructing ingots intended for reduction into hollow wire or tubing, so called, the core employed in my process is of hollow form, as shown in Fig. 4. During the electro-plating step, however, it is desirable to close 90 the ends of the hollow core, A', by plugs or otherwise.

I make no claim to the process of plating flat plates for protecting the core against moisture, nor broadly to electro-plating. I 95 plate substantially cylindrical or seamless members by impact.

Having described my process, what I claim is:

1. The improved process of making cylindrical ingots adapted to be reduced to seamless wire, consisting in depositing upon a metallic rod by electrolysis a film of another metal, and impacting simultaneously all parts of the metal after it is so deposited 105 upon the rod.

2. The improved process of making cylindrical ingots adapted to be reduced to seamless wire, consisting in depositing upon a rod of inferior metal by electrolysis a film of 110

precious metal and impacting simultaneously all parts of the metal after it is so deposited upon the rod.

3. The improved process of making cylindrical ingots adapted to be reduced to seamless wire, consisting in depositing upon a metallic rod by electrolysis a film of another metal, and beating simultaneously all parts of the coated rod.

10 4. The improved process of making cylindrical ingots adapted to be reduced to seamless wire, consisting in depositing upon a metallic rod by electrolysis a film of another metal, and precipitating metal objects by impact against the coated rod.

15 5. The improved process of making cylindrical ingots adapted to be reduced to seam-

less wire, consisting in depositing upon a metallic rod by electrolysis a film of another metal, and precipitating metal objects and 20 soap by impact against the coated rod.

6. The improved process of making ingots adapted to be reduced to seamless wire, which consists in depositing upon a core of base metal a film of another metal and subsequently impacting the outer metal throughout its entire surface for the purpose specified. 25

In testimony whereof I have affixed my signature in presence of two witnesses.

FRANK CUTTER.

Witnesses:

HORATIO E. BELLOW,  
JOSEPH E. BURNS.